

April 12, 1927.

1,624,281

E. R. RUSHTON

PROCESS OF PRODUCING ARSENIC COMPOUNDS

Filed May 28, 1924

FLUENT GASES AND AIR



Inventor

Eugene R. Rushton

334 *Leviathan Bryant Darby*  
Attorneys

## UNITED STATES PATENT OFFICE.

EUGENE R. RUSHTON, OF MADISON, WISCONSIN.

## PROCESS OF PRODUCING ARSENIC COMPOUNDS.

Application filed May 28, 1924. Serial No. 716,441.

The present invention has to do with a new and improved process of producing arsenic compounds, and particularly those arsenates which have been found of great utility as insecticides. The production of such arsenic compounds is, under present methods, expensive, and this, to some extent, militates against their use, because of the prohibitive cost of the product. It is my object to provide a process for the production of such compounds which will efficiently and cheaply give a product having all of the properties necessary to a satisfactory insecticide.

I have discovered that when a material, such as, for example, an oxide of an alkaline earth, is treated with gaseous arsenic trioxide, in the presence of heat and air, that a very complete and rapid combination of the elements necessary to form a satisfactory arsenate results.

While primarily intended to produce a cheap and efficient insecticide, it is obvious that this is only one of the uses to which the product may be put, and this specific application of the arsenate is not, of course, to be taken as in any way limiting my invention, which, as stated, relates to a process of production of the arsenate.

In the drawing herewith is shown diagrammatically a laboratory apparatus by which the process has been successfully carried out.

Referring to the drawings by numbers, a container or flask 10 is provided in which arsenic trioxide or white oxide indicated at A, is placed and heated to vaporization in any suitable manner, as by means of the oil bath 11, which in turn is suitably heated, as by burners 12. The neck 13 of the flask receives the end of a retort 14 suitably supported, and preferably, although not necessarily, so arranged that it may be revolved by any suitable drive mechanism, a driving pulley being shown at one end of the retort, and supporting roller being conventionally shown at each end of the retort. The retort 14 will be charged with the substance to be acted on which may be any suitable metal compound of a group including oxides, hydroxides and carbonates, indicated at B, and I have found that calcium oxide is satisfactory, although it is obvious that any oxide, hydroxide or carbonate of the alkali metals, or alkali earth metals, might be used, cal-

cium oxide being given as one substance which I have used with success.

The retort 14 will be heated in any suitable manner to redness, or to a temperature substantially between 500° C. and 1000° C., 60 the present illustration showing conventionally a battery burner 16 to externally fire the retort.

The delivery end of the retort enters the neck 17 of a container or flask 18 immersed, 65 as here shown, in an oil bath 19, and the vapors coming from the retort and carrying the gases evolved are delivered to the neck of the flask 18.

In order that the product of the process 70 may be carried continuously through the apparatus, I provide a take-off tube 20, which may be connected with any suitable draft inducing means, and, at the opposite end of the retort, I may provide an intake 75 tube 21 so that when the apparatus is functioning, there will be a continuous draft through the retort with air going in through the intake pipe 21, and passing out the take-off pipe 20. This pipe 21 enters the oil 80 bath where it is heated by contact with the oil and as a consequence, air passing through said pipe is likewise heated.

It will be observed that the neck 13 of the container, or flask 10, at the intake end of 85 the retort, is slightly spaced from the walls of the revolving retort, and the draft through the apparatus will induce the flow of a thin film of air at the receiving end of the retort, and, being counter to any pressures created in the retort, will prevent the 90 escape of gas at the receiving end.

At the delivery end of the retort, it will be observed that a similar arrangement is provided, the retort end projecting into the neck 95 17 of the container or flask 18, and being slightly separated therefrom, so that the draft through the take-out pipe 20 will create a flow of air in the form of a thin film between the neck 17 of the flask and the delivery end of the retort, and that any back pressure and escape of gas will be avoided.

I have discovered that in the case of calcium oxide, and oxides, hydroxides and carbonates of the other alkali metals and alkali earth metals, that, following my process, there results a rapid combination of the oxide and the arsenic trioxide gas generated in container 10. The result of this combination seems to be an oxidation of the arsenic 105 110

trioxide to form tri-calcium-orthoarsenate. The equation is represented by the following formula:



The reaction is best obtained at a temperature between 500° C. and 1000° C. and is rapid and complete, as has been ascertained by observing the relatively small amount 10 of arsenic trioxide carried off in the air stream through the take-out pipe 20. The container or flask 18 is intended more particularly to collect any effluent gases, such as uncombined arsenic trioxide, or any of 15 the arsenate which may be entrained in the air stream.

Such product as has been collected in the flask 18, after a retort charge has been subjected to the process, may, of course, be 20 removed therefrom.

In the practice of my process, I have found that it is practicable to calcine limestone directly in the retort 13 to produce the calcium oxide, and in the commercial development 25 of my invention, this might be advantageous, as it would eliminate the step of first calcining limestone, where calcium oxide is the substance used, and then charging it into the retort. A mixture of arsenic trioxide gas and air may be introduced during 30 the calcining operation so that the process may be continuous and while the oxide formed by the calcination is still hot.

As stated, substances other than calcium oxide may be used, in fact, any metals which will combine with the gaseous arsenic trioxide, and particularly an oxide, hydroxide and carbonate of the alkali metal or of the alkali earth metals. For example, potassium 35 oxide, sodium oxide, magnesium oxide, strontium oxide, and barium oxide, and their hydroxides and carbonates are substances which might be substituted in carrying out my process, and there may, of course, be others. I do not, therefore, limit my invention 40 to the particular substances herein specified, since it obviously may be practiced with any substance with which arsenic trioxide will combine to produce the desired product, for example, the oxides, hydroxides and carbonates of such metals as zinc and lead, without changing the principles of the present invention.

The arsenic trioxide may be obtained in any suitable manner, but I have found that by oxidizing calcium arsenite, calcium arsenate and arsenic trioxide is produced, and the trioxide may be recovered and utilized in my process. I have found that at 45 relatively low temperatures, for example 360° C., arsenic trioxide vapor reacts with calcium oxide to form calcium arsenite. The latter is not oxidized to calcium arsenate even in the presence of an excess of air at 50 this temperature. However, if the tempera-

ture is raised to a red heat, or to temperature between 500° C. and 1000° C. in contact with air, some of the arsenic trioxide is driven off as a vapor and combines with the lime and oxygen to form calcium arsenate. 70 My process is equally efficient when this step is employed.

The manner of practicing the process will, it is believed, be clear, and, obviously, it is extremely simple. The container or flask 75 18, is charged with arsenic trioxide, or white oxide, and vaporized. The resulting gaseous arsenic trioxide passes to the rotating retort 14 which has been charged with calcium oxide, or in which limestone has, by 80 the heat of the burners, been converted into calcium oxide. The gaseous arsenic trioxide is brought into intimate contact with the agitated mass of calcium oxide in the retort, and rapidly and effectively combines to form 85 the arsenate. The air draft or suction through the apparatus carries off the uncombined product, and it may be collected in any suitable form of apparatus.

It will be obvious that my illustration to 90 show the steps of my process is simply conventional, and it is not to be taken as restrictive. Various types of apparatus may be used, and a retort inclined to the horizontal and provided with proper feed and discharge devices could be used, so that the charging of the calcium oxide and its passage through the retort would be continuous.

Furthermore, any collecting apparatus may be used to precipitate and collect the product, as, for example, the well known muffling bags, or the equally well known Cottrell precipitating apparatus.

Such variations from this disclosure as amount to simply the skill of the trained mechanician, or chemist, may be made and still be within the range of my invention.

In order that the process may be more easily understood by reference to the drawing, the arsenic trioxide or other arsenic compound is indicated at A. The calcium oxide or substance to be reacted upon is indicated at B. The air stream, as indicated by the arrow, enters through the pipe 21, which is heated by contact with the oil bath, thus preheating the air, and draws the vapors from the chamber 10 to the right into the retort 14, which is preferably rotated and which contains the substance B. The air stream containing the arsenical vapor will react with the substance in the kiln, such as calcium oxide, and a relatively long kiln or tube is employed in order that the reaction may be complete. The temperature is preferably between 500° C. and 1000° C., and the tube is continuously rotated. The air stream passes out through the opposite end of the retort and carries with it the uncombined gases. Some of the effluent products, however, pass into the chamber 18 and

are condensed and recovered, such products being shown at C. The arsenate formed remains in the retort and may be removed as desired. The retort may be so arranged as to deliver the arsenate as formed and the process therefor made continuous.

It will be understood that in the roasting of arseniferous ores, the arsenical gases generated may be embodied in the process of this invention. In such a case, the arsenical gases are passed from the roasting kiln into relation with the oxide, hydroxide or carbonate, and the reaction occurs in the same manner as set forth heretofore. That is to say, an air stream carries the arsenical vapors into contact with the reaction substance in identically the same manner described herein.

I claim:

1. The process which consists in subjecting a substance contributing to the formation of an arsenic compound to an arsenical gas in the presence of oxygen and heat.

2. The process which consists in subjecting a substance contributing to the formation of an arsenic compound to an arsenical gas in the presence of oxygen and at a temperature between 500° C. and 1000° C.

3. The process which consists in subjecting a substance contributing to the formation of an arsenic compound to an arsenical gas in the presence of oxygen and at a temperature between 500° C. and 1000° C., and agitating the mass.

4. The process which consists in subjecting a substance contributing to the formation of an arsenic compound to an air stream containing an arsenical gas in the presence of oxygen and heat.

5. The process of subjecting one of a group of metal compounds which include oxides, hydroxides and carbonates, to the action of arsenical vapor in the presence of heat and air.

6. The process of subjecting one of a group of metal compounds which include oxides, hydroxides, and carbonates to the action of arsenical vapor in the presence of air and at a temperature between 500° C. and 1000° C.

7. The process of subjecting metal compounds which include oxides, hydroxides, and carbonates to the action of arsenical vapor in the presence of air and at a temperature between 500° C. and 1000° C., and agitating the mass.

8. The process of subjecting one of a group of compounds of an alkali forming metal which includes oxides, hydroxides and carbonates to the action of arsenical vapor in the presence of heat and air.

9. The process of subjecting one of a group of compounds of an alkali forming metal which includes oxides, hydroxides and carbonates to the action of arsenical vapor

in the presence of air and at a temperature substantially 500° C. to 1000° C.

10. The process of subjecting one of a group of compounds of an alkali forming metal which includes oxides, hydroxides and carbonates to the action of arsenical vapor in the presence of air and at a temperature substantially 500° C. to 1000° C., and agitating the mass.

11. The process of subjecting a substance contributing to the formation of an arsenic compound to the action of a heated air stream containing an arsenical gas.

12. The process of subjecting one of a group of metal compounds which includes oxides, hydroxides and carbonates to the action of a heated air stream containing arsenical gas.

13. The process of subjecting one of a group of compounds of an alkali forming metal which includes oxides, hydroxides and carbonates to the action of a heated air stream containing an arsenical gas.

14. The process which consists in reacting upon one of a group of metal compounds which includes oxides, hydroxides, and carbonates with arsenical vapors generated by the roasting of arseniferous ores in the presence of heat and air.

15. The process which consists in reacting upon one of a group of metal compounds which includes oxides, hydroxides and carbonates with arsenical vapors generated by the roasting of arsenical ores, such vapors being drawn in an air stream and reaction taking place at a temperature of substantially 500° C. to 1000° C.

16. The process which consists in reacting upon one of a group of metal compounds which includes oxides, hydroxides and carbonates with arsenical vapors generated by the roasting of arsenical ores, such vapors being drawn in a heated air stream and reaction taking place at a temperature of substantially 500° C. to 1000° C., and agitating the mass.

17. The process which consists in reacting upon one of a group of compounds of an alkali forming metal which includes oxides, hydroxides and carbonates with arsenical vapors generated by the roasting of arseniferous ores in the presence of heat and air.

18. The process which consists in reacting upon one of a group of compounds of an alkali forming metal which includes oxides, hydroxides and carbonates with arsenical vapors generated by the roasting of arseniferous ores, such vapors being entrained in an air stream and reaction taking place at a temperature of substantially 500° C. to 1000° C.

19. The process which consists in reacting upon one of a group of compounds of an alkali forming metal which includes oxides, hydroxides and carbonates with arsenical va-

- 5      pores generated by the roasting of arseniferous ores, such vapors being entrained in a heated air stream and reaction taking place in the presence of air with the mass at red heat and with agitation.
- 10     20. The process of reacting upon one of a group of compounds which includes oxides, hydroxides and carbonates with arsenical vapors, the combination taking place throughout a prolonged period in the presence of heat and air.
- 15     21. The process of reacting upon one of a group of metal compounds which include oxides, hydroxides and carbonates with arsenical vapors, the combination taking place through a prolonged period in the presence of air and at a temperature of substantially 500° C. to 1000° C.
- 20     22. The process of reacting upon one of a group of compounds of an alkali forming metal which includes oxides, hydroxides and carbonates with arsenical vapors, the combination taking place through the prolonged period in the presence of heat and air.
- 25     23. The process of reacting upon one of a group of calcium compounds which include oxides, hydroxides and carbonates with arsenical vapors, the combination taking place through a prolonged period in the presence of heat and air.
- 30     24. The process of acting upon one of a group of metal compounds which include oxides, hydroxides and carbonates with arsenical vapors entrained in an air stream, the combination taking place through a prolonged period in the presence of heat and air.
- 35     25. The process of acting upon one of a group of metal compounds which include oxides, hydroxides and carbonates with arsenical vapors entrained in an air stream, the combination taking place through a prolonged period in the presence of heat and air, and with agitation of the mass.
- 40     26. The process of subjecting calcium compounds of the group which include oxides, hydroxides and carbonates to the action of an arsenical gas in the presence of heat and air.
- 45     27. The process of subjecting calcium compounds of the group which include oxides, hydroxides and carbonates to the action of an arsenical gas in the presence of heat and air and agitating the mass.
- 50     28. The process of subjecting calcium compounds of the group which includes oxides, hydroxides and carbonates to the action of an air stream containing arsenical gas in the presence of heat and air.
- 55     29. The process of subjecting calcium compounds of the group which include oxides, hydroxides and carbonates to the action of an arsenical gas in the presence of air and at a temperature of between 500° C. to 1000° C.
- 60     30. The process of subjecting calcium compounds of the group which include oxides, hydroxides and carbonates to the action of an arsenical gas in the presence of air and at a temperature of between 500° C. and 1000° C., and agitating the mass.
- 65     31. The process of subjecting calcium compounds of the group which include oxides, hydroxides and carbonates to gaseous arsenic trioxide in the presence of heat and air.
- 70     32. The process of subjecting calcium compounds of the group which include oxides, hydroxides and carbonates to an air stream containing gaseous arsenic trioxide in the presence of heat and air.
- 75     33. The process of subjecting calcium compounds of the group which include oxides, hydroxides and carbonates to the action of an air stream containing gaseous arsenic trioxide, the reaction taking place through a prolonged period, and in the presence of oxygen and heat.
- 80     34. The process of subjecting calcium compounds of the group which include oxides, hydroxides and carbonates to gaseous arsenic trioxide in the presence of air and at red heat.
- 85     35. The process of subjecting calcium compounds of the group which include oxides, hydroxides and carbonates to gaseous arsenic trioxide in the presence of air and at red heat and agitating the mass.
- 90     36. The process which consists in subjecting calcium compounds which include oxides, hydroxides and carbonates to the action of gaseous arsenic trioxide in the presence of heat and air while the mass is being agitated.
- 95     37. The process which consists in calcining a carbonate and subjecting the hot mass to an arsenical vapor in the presence of air.
- 100     38. The process which consists in calcining a metal carbonate and subjecting the hot mass to an air stream containing arsenic trioxide at a temperature of substantially 500° C. to 1000° C. while agitating the mass.
- 105     39. The process which consists in calcining a carbonate of an alkali forming metal and subjecting the mass at red heat to an arsenical vapor in the presence of air.
- 110     40. The process which consists in calcining an alkali forming metal and subjecting the hot mass to an air stream containing arsenic trioxide at a temperature of substantially 500° C. to 1000° C., and agitating the mass.
- 115     41. The process which consists in subjecting calcium compounds of a group which includes oxides, hydroxides and carbonates to the action of an air stream containing arsenical vapors produced in the roasting of arseniferous ores at a temperature of substantially 500° C. to 1000° C.
- 120     42. The process which consists in calcin-
- 125     130

- ing a carbonate and passing an air stream containing arsenical vapors produced from the roasting of arseniferous ores over the calcined carbonate, and maintaining the mass 5 agitated at a temperature between 500° C. and 1000° C.
43. The process which consists in subjecting calcium compounds of a group which include hydroxides, carbonates and oxides to 10 the action of a heated air stream containing arsenical vapors at a temperature of substantially 500° C. to 1000° C.
44. The process of forming arsenates which consists in reacting upon calcium oxide in
- the presence of air with arsenic trioxide 15 vapor at a temperature of 360° C. and thereafter subjecting the mass to temperatures between 500° C. and 1000° C. in the presence of air.
45. The process of producing calcium arsenate which consists in subjecting calcium oxide while in a state of agitation to the action of arsenic trioxide in the presence of oxygen and heat.

In testimony whereof I have hereunto set 25 my hand.

EUGENE R. RUSHTON.